

## 1

3,070,421

ALUMINUM, CHROMIUM, AND GALLIUM  
TELLURATES

Gerhard Bayer, Hinteregg, Zurich, Switzerland, assignor  
to Owens-Illinois Glass Company, a corporation of  
Ohio  
No Drawing. Filed Dec. 7, 1960, Ser. No. 74,226  
4 Claims. (Cl. 23—50)

This invention relates to new metal tellurates. In a more specific aspect, the invention relates to new compounds of the type  $A_2TeO_6$ , wherein the A atoms have a valence of 3 and the tellurium atoms have a valence of 6, and wherein A is Cr, Al, or Ga.

Rutile-type compounds can be classified into three groups:  $A^{4+}O_2$ ,  $A^{3+}B^{5+}O_4$ ,  $A^{2+}B_2^{5+}O_6$ . The prototype  $A^{4+}O_2$  compound is rutile,  $TiO_2$ .  $A^{3+}B^{5+}O_4$  compounds have the same unit cell and are typified by statistical distribution of the cations in the lattice. Examples include tantalates, such as  $CrTaO_4$ , and antimonates, such as  $AlSbO_4$ .  $A^{2+}B_2^{5+}O_6$  compounds have the trirutile structure as reported by Goldschmidt et al., "Geochemische Verteilungsgesetze der Elemente: VI, Über die Kristallstrukturen vom Rutiletypus" (Geochemical Distribution Law of the Elements: VI, Crystal Structure of Rutile Type With Remarks on Geochemistry of the Bivalent and Quadrivalent Elements), Skrifter Norske Videnskaps-Akad. Oslo, Mat-Nat. Kl., No. 1, 21 pp. (1926); p. 18.

The rutile and trirutile structures are closely related. The unit cell of the trirutile structure corresponds to three unit cells of the monorutile structure, except that the Ti positions are occupied in a regular way by  $A^{2+}$  and  $B^{5+}$  ions. Both belong to the space group  $P4/mm$ . Prior to my invention only compounds of the general type  $A^{2+}B_2^{5+}O_6$  have been found to have the trirutile structure (Anders Bystrom, Brita Hok, and Brian Mason, "Crystal Structure of Zinc Metantimonate and Similar Compounds," Arkiv. Kemi, Mineral. Geol., 15B (4) 1-8 (1941); Brian Mason and C. J. Vitaliano, "Bystromite, Magnesium Antimonate, a New Mineral," Amer. Mineralogist, 37, 53-57 (1952)).

An object of the present invention is to provide new tellurium compounds containing hexavalent tellurium.

Another object of the invention is to provide new compounds capable of existing in an unusual inverse trirutile-type structure.

Other objects of the invention will become apparent from a study of the accompanying disclosure.

According to the present invention, I have now discovered new metal tellurates of the formula  $A_2TeO_6$ , wherein the valence of the A atom is 3 and the valence of the tellurium is 6. In contrast to trirutile compounds disclosed in the published literature, my present compounds have the general formula  $A_2BO_6$ .

The general formula for this compound is in contrast to the general formula  $AB_2O_6$  for a normal trirutile compound. The lattice positions of A and B ions are therefore interchanged and the structure of the present crystalline compounds can be interpreted as an "inverse trirutile structure." These compounds can be regarded as a superlattice of rutile, with regular distribution of the  $A^{3+}$  and  $Te^{6+}$  ions in the tripled rutile cell.

## 2

With B representing  $Te^{6+}$ , the sequence of atomic layers in these compounds is . . . AABAABAABAAB . . . ( $A=Al$ ,  $Ga$  or  $Cr$ ;  $B=Te$ ) as compared to

. . . ABBABB . . .

in normal trirutile compounds. Disregarding the oxygens (the 0-parameter should be fairly constant in all compounds), the relative intensities of the same type of X-ray reflection will be determined by the arrangement and the diffracting power of the cations. For the first reflection 002 waves from all the 3-valent ions (Al, Ga, or Cr) oppose to some extent those from the Te-ions. Therefore, this reflection is weakest for the compound containing  $A(3+)$  with the highest diffracting power, that is,  $Ga_2TeO_6$ . Values of the atomic scattering factors for this reflection are listed below and compared to the relative intensities.

|             | $hkl$ | $d$   | $\frac{\sin \theta}{\lambda} = \frac{1}{2d}$ | $f(A^{3+})$ | $I/I_1$ |
|-------------|-------|-------|----------------------------------------------|-------------|---------|
| $Al_2TeO_6$ | 002   | 4.35  | 0.115                                        | 9.61        | 34      |
| $Ga_2TeO_6$ | 002   | 4.48  | 0.111                                        | 27.3        | 7       |
| $Cr_2TeO_6$ | 002   | 4.495 | 0.111                                        | 21.0        | 12      |

$(f_{Te} \sim 47)$

The relatively high diffracting power of  $Te(6+)$  is "reduced" by the diffracting power of the 3-valent ion. 30 Therefore, the reflection 002 is strongest in the compound  $Al_2TeO_6$ . The same is true for the next reflection 101. Also, here planes of Te are interleaved by planes of A-ions ( $A=Al$ ,  $Ga$ ,  $Cr$ ). The higher the diffracting power of the A-ion, the weaker should be the intensity of this reflection. 35 This is in complete agreement with the observed intensities. In all such cases, where "homogeneous" planes (occupied either by  $Te(6+)$  or by  $A(3+)$ ) are concerned, the intensities of the reflections decrease in the order  $I(Al_2TeO_6) > I(Cr_2TeO_6) > I(Ga_2TeO_6)$ . This is true for 002, 101, 112, 004, 202, 211, and so on. In other cases, where the planes are occupied by both kinds of cations, the reverse order for the relative intensities is found. For these "heterogeneous" planes, the intensity of reflections is proportional to the mean value of  $(f_{Te} + 2f_A)^2$  and therefore highest for  $Ga_2TeO_6$  and lowest for  $Al_2TeO_6$ . Examples are 103 and 200.  $Al_2TeO_6$  has the smallest lattice constant of all known trirutile compounds.

Each of these compounds was prepared by mixing equimolar proportions of the respective  $A_2O_3$  compound with  $TeO_2$ . The respective oxides were finely divided powders of less than 20 mesh. They were intimately admixed, pressed to a cohesive shape and then fired in an oxidizing (air) atmosphere at 650-700°C. for a period of 20 hours. The  $Al_2O_3$  and  $Cr_2O_3$  were available, but the  $Ga_2O_3$  had to be prepared from metallic gallium by dissolving in diluted  $H_2SO_4$ , precipitating with  $NH_4OH$ , and then calcining.

The oxidizing atmosphere used in firing these  $A_2TeO_6$  compounds of the invention by the solid-state reaction is necessary in order to convert the tellurium to the hexavalent state. Table I shows the X-ray powder diffraction data, the calculated lattice constants, and the calculated densities of each of the new compounds so prepared.

TABLE I  
X-Ray Powder Diffraction Data

| Al <sub>2</sub> TeO <sub>6</sub> |                  |            | Ga <sub>2</sub> TeO <sub>6</sub> |                  |            | Cr <sub>2</sub> TeO <sub>6</sub> |                  |            |
|----------------------------------|------------------|------------|----------------------------------|------------------|------------|----------------------------------|------------------|------------|
| <i>d</i>                         | I/I <sub>1</sub> | <i>hkl</i> | <i>d</i>                         | I/I <sub>1</sub> | <i>hkl</i> | <i>d</i>                         | I/I <sub>1</sub> | <i>hkl</i> |
| 4.35                             | 34               | 002        | 4.48                             | 7                | 002        | 4.495                            | 12               | 002        |
| 3.94                             | 86               | 101        | 4.05                             | 18               | 101        | 4.06                             | 28               | 101        |
| 3.12                             | 100              | 110        | 3.21                             | 100              | 110        | 3.21                             | 100              | 110        |
| 2.54                             | 29               | 112        | 2.61                             | 5                | 112        | 2.61                             | 9                | 112        |
| 2.42                             | 51               | 103        | 2.49                             | 65               | 103        | 2.50                             | 55               | 103        |
| 2.21                             | 10               | 200        | 2.27                             | 18               | 200        | 2.272                            | 13               | 200        |
| 2.172                            | 4                | 004        | 2.24                             | 2                | 004        | ---                              | ---              | ---        |
| 2.12                             | 14               | 113        | 2.185                            | 7                | 113        | 2.19                             | 9                | 113        |
| 1.97                             | 12               | 202        | 2.025                            | 4                | 202        | 2.03                             | 6                | 202        |
| 1.93                             | 19               | 211        | 1.98                             | 5                | 211        | 1.98                             | 8                | 211        |
| 1.78                             | 9                | 114        | 1.836                            | 3                | 114        | 1.84                             | 3                | 114        |
| 1.634                            | 47               | 213        | 1.68                             | 52               | 213        | 1.68                             | 41               | 213        |
| 1.618                            | 6                | 105        | 1.666                            | 4                | 105        | ---                              | ---              | ---        |
| 1.56                             | 12               | 220        | 1.605                            | 15               | 220        | 1.605                            | 12               | 220        |
| 1.55                             | 4                | 204        | 1.595                            | 3                | 204        | ---                              | ---              | ---        |
| 1.475                            | 3                | 222        | 1.51                             | 2                | 222        | ---                              | ---              | ---        |
| 1.45                             | 3                | 301        | 1.492                            | 8                | 301        | 1.50                             | 6                | 301        |
| 1.449                            | 7                | 006        | 1.49                             | 6                | 006        | 1.492                            | 3                | 006        |
| 1.40                             | 7                | 310        | 1.435                            | 12               | 310        | 1.436                            | 7                | 310        |
| 1.33                             | 4                | 312        | 1.366                            | 2                | 312        | 1.37                             | 3                | 312        |
| 1.314                            | 17               | 303        | 1.33                             | 20               | 303        | 1.356                            | 8                | 303        |
| 1.308                            | 6                | 116        | 1.346                            | 10               | 116        | 1.352                            | 12               | 116        |
| 1.27                             | 2                | 224        | ---                              | 5                | 206        | 1.25                             | 3                | 206        |
| 1.21                             | 4                | 206        | 1.246                            | 5                | 206        | ---                              | ---              | ---        |

Tetragonal unit cell, space group of P4/mnm, Z=2  
LATTICE CONSTANTS (A.U.)

|               |      |       |
|---------------|------|-------|
| $a_0 = 4.445$ | 4.54 | 4.545 |
| $c_0 = 8.70$  | 8.97 | 8.99  |
| $D^* = 5.37$  | 6.52 | 5.85  |

\*Density (g./ccm.) (from X-ray data).

Each of the compounds so prepared was stable up to a temperature of about 730° C. At this temperature and higher after long heating the compounds begin to decompose. Each of the compounds is insoluble in water and most acids (no change of the X-ray pattern).

The color of the aluminum and gallium compounds

was white while the chromium compound was a gray-green.

The new compounds find particular application as pigments in ceramic glazes, enamels, paints and dyes. They are also useful as pigments in plastics; for instance, they can be incorporated as powders in plastics, such as polyethylene or polystyrene, in amounts from 0.5 to 10 weight percent, or even higher.

As a specific example of a paint formulation incorporating the present pigments, the following is illustrative.

| Ingredient:                                                                                               | Lbs. |
|-----------------------------------------------------------------------------------------------------------|------|
| Al <sub>2</sub> TeO <sub>6</sub> , Cr <sub>2</sub> TeO <sub>6</sub> , or Ga <sub>2</sub> TeO <sub>6</sub> | 300  |
| Zinc oxide                                                                                                | 25   |
| Long-oil soya alkyd resin (60% nonvolatile)                                                               | 480  |
| 15 Mineral spirits                                                                                        | 181  |
| Cobalt naphthenate (6% Co)                                                                                | 3    |
| Lead naphthenate (24% PbO)                                                                                | 3    |
| Calcium naphthenate (4% Ca)                                                                               | 2    |
| Total                                                                                                     | 994  |

While the compounds of the invention normally exist in the inverse trirutile-type crystalline state when pure, they can also form solid solutions in other compounds.

25 As will be evident to those skilled in the art, various modifications of this invention can be made or followed in the light of the foregoing disclosure and discussion without departing from the spirit and scope of the disclosure or from the scope of the claims.

I claim:

30 1. A compound of the formula A<sub>2</sub>TeO<sub>6</sub>, wherein A is selected from the group consisting of aluminum, gallium and chromium.

2. The compound Cr<sub>2</sub>TeO<sub>6</sub>.

3. The compound Al<sub>2</sub>TeO<sub>6</sub>.

35 4. The compound Ga<sub>2</sub>TeO<sub>6</sub>.

References Cited in the file of this patent

Mellor: Comprehensive Treatise on Inorganic and Theoretical Chemistry, Longmans, Green and Co., New York, vol. XI, pages 88, 89, 96 and 97.